

## UNITED STATES PATENT OFFICE

2,224,711

## ABRASIVE

Arthur J. Weinig, Golden, Colo.

No Drawing. Application January 16, 1939,  
Serial No. 251,132

3 Claims. (Cl. 51—307)

This invention relates to a precision abrasive and to the process of manufacturing the same.

The finest abrasive materials at present on the market are either too coarse, too evenly graded, or too harsh to produce a microscopically sharp, cutting edge of high precision; or else they are so soft and fine as to require great time and labor to produce a satisfactory cutting edge. Present abrasives are also usually incorporated in a 10 greasy, oily, or waxy binder which causes glazing of the honing surface so that uniformity of edge is impossible.

The principal object of this invention is to produce an extremely finely divided abrasive of fast 15 but tempered cutting qualities which will be suitable for sharpening precision instruments of the type which require an extremely sharp cutting edge such as surgical instruments, microtome knives, razors, etc. and to provide a process for 20 manufacturing the abrasive which will be simple and economical and which will produce a uniformly excellent product.

Another object of the invention is to provide an abrasive in which all greasy, oily, or oleaginous 25 binders are eliminated so that the final product will be a dry, fine abrasive in powdered or stick form which will not be subject to self-classification, separation, or stratification and which 30 will permanently maintain a uniformity of material throughout an entire batch without the objectionable features of a greasy or waxy substance.

A still further object of the invention is to provide an abrasive which will cling uniformly 35 over the entire honing surface without the use of greases, waxes, oils, or soaps. In fact, in the present invention, in the final product there is no water, salt, rosin, wax, oil, soap, or other similar vehicle for binding purposes. These have 40 been eliminated to avoid their undesirable lubricating properties yet all their desirable qualities have been maintained by so forming the product that it acts as a self-binding and self-clinging product, and one that can be operated without 45 glazing.

One of the principal uses for the product has 50 been found to be the grinding of surfaces such as mineral surfaces, meteoric surfaces, microscope slides, and the like for microscopic study. For such a study any surface abrasions or 55 scratches, would be objectionable due to the great magnification thereof and for this purpose none of the ordinary grinding compounds would be of any value. The improved material, however, is not limited to this specific use but has been found

to be of great value in sharpening precision cutting blades such as microtome blades to an exceedingly fine smooth cutting edge.

Abrasives such as the finest grades available on the market of optical emery, flours of silicon carbide, boron carbide, tungsten carbide, alumina and garnet, are fast cutting. The main grain sizes range from 80 to 20 microns. They do not however produce the microscopically polished surface necessary for microtome or microscopic 10 purposes. On the other hand, the finer soft abrasives, such as the metallic oxides generally known as crocus, red and black rouge, etc. do produce a high polish but the cutting action is very slow and they are incapable of removing 15 the bilge or roundness that develops along the sides of cutting edges through long use.

This invention comprises a dry abrasive powder having all the desirable qualities of a harsh abrasive combined with all the desirable qualities of a soft abrasive. The preferred form of the improved abrasive is an intimately intermixed compound of two differing abrasive materials of differing hardness and differing coarseness, so arranged that the preponderance of the 25 coarser grains will be of the harder constituents while the preponderance of the finer grains will be of the softer constituent. The softer constituent is ground to a sufficient fineness to act as a dry binder for maintaining the coarser grains 30 evenly, uniformly, and permanently distributed throughout the product and so that its excessive fineness will impart a clinging or adhesive action to cause the composition to adhere to surfaces in the nature of the clinging action of dry 35 chalk.

## Process

The finest available hard abrasive products now obtainable on the market such as silicon carbide or/and aluminum oxide hereafter called 40 the abrasive is subjected to wet or dry grinding in a pebble mill. The grinding media consists of pebbles of flint or chalcedony. During the grinding, the flint pebbles wear down more rapidly 45 than the harder abrasive and produce a pulp consisting of an abundance of extremely fine siliceous powder mixed with a lesser amount of fine grains of the harder abrasive.

The grinding reduces a majority of the original silicon carbide grains to from 20 microns to 1 micron in size. The major portion of the flint worn from the pebbles attains a grain size of from 1 to 5 microns although there will also be considerable flint in sizes reaching up to 20 55

microns. All of the grain sizes above 20 microns are rejected and if the amount of flint of 5 microns or less is too great, a portion of it is also rejected.

5 The powder remaining after the above rejections has all the rapid cutting qualities of the silicon carbide or aluminum oxide and in addition the harshness has been removed or tempered by the buffer action of the fine flint grains. The 10 powder thus produced cuts rapidly and yet maintains smooth, highly polished, surfaces which can be brought to an extremely thin edge without bilge.

To prevent any possibility of segregation or 15 stratification and to further the adherence of the powder to a honing surface such as a leather strop and to otherwise improve the soft, yet rapid, cutting action of the product, it is preferred to incorporate the combined powders into a dry gel, 20 preferably insoluble copper hydroxide, although the insoluble hydroxides of aluminum, zinc, and iron and vegetable gums are also suitable. The method of applying the gel is preferably as follows:

#### 25 First decant

The combined, ground abrasive is agitated in water in a shallow tank. If impure water or other causes produce flocculation a suitable deflocculating agent such as tannic acid is added. The pulp is allowed to repose quietly until by test or calculation all grain sizes above 5 microns have settled below a pre-determined level in the tank. The pulp above this level is then siphoned or decanted off. The pulp in the decant will now contain the 35 major portion, but not all, of the particles of 5 microns or less. A solution of copper sulfate is now added to the latter pulp and the mixture is well agitated. An alkali, such as a sodium hydroxide solution, is now carefully added with continued agitation until the copper is substantially all precipitated as copper hydroxide in the pulp after which the pulp is allowed to repose quietly. The large flocs of gel in which the particles of 45 the abrasive and flint are entrapt now settle rapidly and, as soon as settlement is complete, the supernatant clear water is siphoned off and the residual thickened pulp is filtered and dried.

The product thus derived, herein referred to as 50 the "first decant," will be largely fine flint (5 microns or less). It is reserved for blending with a second decant material.

#### Second decant

55 The coarser pulp remaining in the original tank, below the decanted level (exceeding 5 microns), is again agitated in water, a deflocculant is added if necessary, and is then allowed to repose and settle until by test or calculation the 60 particles larger than 20 microns have settled out below a predetermined level. The pulp above this level is then decanted and treated with copper sulfate, alkali, settled, filtered and dried as was done in the first decantation. This second decantation 65 is repeated in all detail, usually four times, until continued decantations do not yield substantial amounts of sized material below 20 microns size. We now have a product consisting in the main 70 of the abrasive flour of less than 20 microns grain

size which will be designated the "second decant."

#### Final combination

The first and second decants are now intimately intermixed in the dry state to produce the 5 final abrasive product. The mixture is carefully tested and controlled by placing samples on a smooth, level, leather strop and then stropping a section of microtome blade. If there is a harsh cutting action, which can be detected after a little trial and experience, an additional amount of the first decant is added to the compound until the test shows the harshness is eliminated. The final product is then moistened, thoroughly remixed, and dried. It may be marketed as a loose 10 dry powder or may be pressed into cakes or sticks by pressure. Such sticks or cakes are convenient for dispensing the abrasive as a chalk like product.

The remaining settled material in the tank 15 containing the grains above 20 microns is returned with a new charge of the abrasive flour to the pebble mill for regrinding and retreatment.

Experience will in time teach one to so regulate the time of grinding that the proper proportion of fine flint material will be produced in the pebble mill so that the initial separation of the 5 micron sizes in a first decant will not be necessary and all decants then can be conducted simply for the separation of material coarser than 20 30 microns.

The excess fine flint which has been rejected after the grinding will contain a certain amount of fine carborundum which, of course, would be valuable in the final product.

This carborundum may be separated from the flint and recovered by froth flotation in water. Pine oil or cresylic acid may be used as a frothing reagent and any suitable collecting reagent such as a fatty acid or its soaps may be used. It has been found that carborundum grains up to 35 mesh can be readily removed from the flint by this froth flotation method.

While a preferred form of product has been described in some detail for use in sharpening instruments requiring a very fine cutting edge together with the preferred process of producing the same, it is to be understood that the invention is not limited to the precise ingredients nor to the precise procedure described except in so far as such limitations are included in the appended claims in which it is the intention to claim all novelty inherent in the invention with due regard to the prior art.

Having thus described the invention what is claimed and desired secured by Letters Patent is:

1. A dry abrasive for fine grinding comprising: a dry mixture of powdered silicon carbide, powdered flint, and precipitated copper hydroxide 80 the grain size of the silicon carbide not exceeding 20 microns and the grain size of the flint not exceeding 5 microns in size.

2. A dry abrasive for fine grinding comprising: a dry mixture of powdered silicon carbide, powdered flint, and precipitated copper hydroxide.

3. An abrasive for fine grinding comprising: powdered silicon carbide; powdered flint; and a precipitated metal hydroxide.

ARTHUR J. WEINIG.